

# UNITED STATES PATENT OFFICE.

JAMES V. Z. BLANEY, OF CHICAGO, ILLINOIS.

## IMPROVEMENT IN PROCESSES FOR RESTORING WRITING OR PRINTING ON CHARRED PAPER.

Specification forming part of Letters Patent No. 121,321, dated November 28, 1871.

*To all whom it may concern:*

Be it known that I, JAMES V. Z. BLANEY, of Chicago, Cook county, State of Illinois, have invented a new and useful Process for Rendering Legible Printed and Written Matter upon Paper which has been wholly or partially charred by fire.

The charred paper is to be first separated into single leaves, and then immersed in a solution of a soluble compound of silver or copper for such a time as may be required to render the printing or writing sufficiently legible. A solution of the nitrate of silver containing forty (40) grains of that salt to one fluid ounce of distilled water is preferred. If the restoration is only required to be made on one side of the sheet, the solution may be applied with a brush, or by floating the paper upon the surface of the liquid.

The process succeeds best in a dark or a feebly-lighted room. After sufficient legibility has been

attained the paper should be soaked for some time in pure water to remove the excess of the salt used—in the case of silver salts a dilute solution of hyposulphite of soda or of cyanide of potassium may be used—after which the paper may be exposed to the light, and, when dry, covered with a transparent mucilage or varnish for preservation.

What I claim as my invention is—

The use of the soluble compounds of silver and of copper for the restoration, temporarily or permanently, of writing or printing on paper which has been wholly or partially charred by fire, such charring having rendered such writing or printing wholly or partially illegible.

JAS. V. Z. BLANEY.

Witnesses:

W. M. R. PAGE,  
R. BIDDLE ROBERTS.

(35)